

Aug. 23, 1960

J. D. BATCHELOR ET AL  
METHOD FOR MAINTAINING HIGH LEVEL OF ACTIVITY  
FOR SUPPORTED MANGANESE OXIDE ACCEPTORS  
FOR HYDROGEN SULFIDE

2,950,229

Filed Oct. 28, 1957

2 Sheets-Sheet 1



FIG. 1



FIG. 3

INVENTORS  
JAMES D. BATCHELOR  
GEORGE P. CURRAN  
EVERETT GORIN

BY *Harry B. Keck*  
ATTORNEY

Aug. 23, 1960

**1960 J. D. BATCHELOR ET AL  
METHOD FOR MAINTAINING HIGH LEVEL OF ACTIVITY  
FOR SUPPORTED MANGANESE OXIDE ACCEPTORS  
FOR HYDROGEN SULFIDE**

2,950,229

Filed Oct. 28, 1957

2 Sheets-Sheet 2



**FIG. 2**

INVENTORS  
AMES D. BATCHELOR  
GEORGE P. CURRAN  
VERETT GORIN

BY EVERETT GORIN  
*Harry B. Kack*  
ATTORNEY

1

2,950,229

## METHOD FOR MAINTAINING HIGH LEVEL OF ACTIVITY FOR SUPPORTED MANGANESE OXIDE ACCEPTORS FOR HYDROGEN SULFIDE

James D. Batchelor, Bethel Park, and George P. Curran and Everett Gorin, Pittsburgh, Pa., assignors to Consolidation Coal Company, Pittsburgh, Pa., a corporation of Pennsylvania

Filed Oct. 28, 1957, Ser. No. 692,897

12 Claims. (Cl. 202—31)

The present invention relates to a process for maintaining a high state of activity in supported manganese oxide acceptors for hydrogen sulfide. More particularly, it relates to a process for removing sulfur contamination from carbonaceous solid materials by treatment with hydrogen in the presence of manganese oxide-type solid acceptors for hydrogen sulfide.

Such sulfur removal processes for carbonaceous solid fuels have been described in copending U.S. patent application S.N. 527,705, now U.S. Patent 2,824,047, filed August 11, 1955, by Everett Gorin, George P. Curran and James D. Batchelor, assigned to the assignee of the present invention. A further process relating to sulfur removal and calcining of carbonaceous solid fuel briquets has been described in copending U.S. patent application S.N. 635,278, filed January 22, 1957, and since abandoned, and in copending U.S. patent application S.N. 1,837, filed January 5, 1960, both by James D. Batchelor, Everett Gorin, George P. Curran and Robert J. Friedrich, both assigned to the assignee of the present invention.

The presence of sulfur in carbonaceous solid fuels limits their use in metallurgical applications. Accordingly, most metallurgical fuels are obtained by employing low sulfur content starting materials, e.g., low sulfur coal is converted to low sulfur metallurgical coke. Sulfur removal processes of the type described in the aforementioned patent applications permit the use of high sulfur content fuels as starting materials for preparing low sulfur content carbonaceous fuels for metallurgical use. For example, the sulfur removal process may be provided as a treatment for the solid residue (termed char) resulting from low temperature carbonization of bituminous coal. Where fluidized low temperature carbonization processes are used, the finely divided, low density, porous char product is particularly amenable to those desulfurization treatments. The desulfurization treatment can be applied to any non-caking carbonaceous solid fuel such as cokes and chars. Coke from coal and hydrocarbonaceous residues (pitch coke), coke breeze, low temperature carbonization char from coal and lignite are exemplary. The processes cannot be applied to caking carbonaceous solid fuels such as caking coal since the thermal treatment encompassed in such processes would cause these materials to become sticky and form coked masses which would bind the acceptor solids, thus preventing their recovery for reuse in the process. Further the resulting coke would be contaminated with the acceptor solids; any sulfur transferred from the carbonaceous fuels to the bound acceptor solids would remain in the solid coke. The processes, however, are applicable to the desulfurization of carbonaceous briquets which may contain caking coal inter alia provided the thermal treatment is conducted to avoid severe caking and accompanying formation of large coke masses.

In the aforementioned copending application S.N. 527,705 solid carbonized carbonaceous fuels are desulfurized by treatment at elevated temperatures in the

2

presence of hydrogen and a solid acceptor for hydrogen sulfide. A preferred acceptor in this process is one containing manganese oxide impregnated on an inert support.

According to that process, carbonaceous solid fuels containing sulfur are mixed with a solid material (termed an "acceptor") which is capable of absorbing hydrogen sulfide. The mixture is treated with hydrogen gas at a temperature above about 1100° F. whereby the hydrogen gas combines with the contaminating sulfur to form hydrogen sulfide; the hydrogen sulfide is absorbed in situ by the acceptor. Since the hydrogen sulfide is absorbed almost instantly upon formation, there is only a negligible partial pressure of hydrogen sulfide in the desulfurization zone for inhibiting the reactions whereby sulfur is removed from the carbonaceous solid fuels. The reaction mixture of solids is separated into (a) product desulfurized carbonaceous solid fuels and (b) the solid acceptor containing absorbed sulfur. The acceptor may be regenerated and heated by contact with air to restore its hydrogen sulfide acceptor properties through elimination of previously absorbed sulfur. The heated regenerated acceptor, when mixed with relatively cool carbonaceous solid fuels preferably provides the heat necessary to raise the solids reaction mixture to a desulfurization temperature.

Where the sulfur-containing carbonaceous solid fuel is in the form of finely divided particles (e.g., fluidized low temperature carbonization char, petroleum coke and the like), the acceptor preferably is larger in size to facilitate separation of desulfurized fuel from the sulfided acceptor. When the sulfur-containing carbonaceous solid fuel is in the form of relatively large agglomerate masses, such as briquets, the acceptor preferably is in the form of finely divided fluidizable size particles to improve contacting efficiency and to facilitate separation of desulfurized fuel from the sulfided acceptor.

Carbonaceous solid fuels contain sulfur in at least three forms. Some of the sulfur exists as readily removable sulfur which is organically bound in the carbonaceous fuel. This organically bound sulfur can be removed from the carbonaceous solid fuels rather easily by contact with hydrogen. If the readily removable, organically bound sulfur is represented as  $-\text{C}=\text{S}$ , the desulfurization reaction may be represented as follows:



Some of the sulfur exists as inorganically bound sulfur usually in the form of metallic (principally iron) sulfide. This sulfur may be removed rather readily by treating the carbonaceous solid fuel with pure hydrogen gas. The reaction (assuming iron sulfide) is as follows:



The equilibrium ratio for this reaction



is very low. Hence small quantities of hydrogen sulfide in the gas phase will inhibit the transfer of sulfur from the solid to the gas. At 1350° F., for example, 0.12 volume percent of hydrogen sulfide in the hydrogen gas is the equilibrium value. At 1600° F., 0.28 volume percent of hydrogen sulfide in the hydrogen gas is the equilibrium value. Thus in order to remove inorganically bound sulfur effectively, the ratio of



must be maintained at an extremely low value, i.e., nearly pure hydrogen must be used.

A further type of sulfur existing in the solid carbona-

ceous fuels is identified as "difficultly removable sulfur" which is principally organically bound. This type of sulfur exists in the form of refractory organic material and various inorganic sulfides. While this sulfur theoretically can be removed by treatment of the carbonaceous solid fuels with pure hydrogen gas, nevertheless, even minute traces of hydrogen sulfide are sufficient to inhibit the transfer of sulfur from the solids to the gas. Removal of the difficultly removable sulfur is not practicable under feasible processing conditions.

The ultimate desulfurization which can be achieved at any temperature depends upon the ratio of



in the treating gases without regard to the absolute pressure of the reaction system. While greater absolute pressure increases the rate of desulfurization, it does not affect the ultimate level of sulfur in the treated solids. In accordance with these findings, satisfactory desulfurization rates may be achieved at temperatures above about 1100° F. with atmospheric pressure. Higher pressure accomplishes the same desulfurization in shorter time. A preferred pressure range for the desulfurization is about 1 to 6 atmospheres absolute.

It is possible to maintain a low value for the ratio



by employing enormous quantities of hydrogen as a treating gas. For example, the use of 1000 molar volumes of pure hydrogen gas in removing one mol of sulfur would create an environment containing 0.10 volume percent of  $\text{H}_2\text{S}$  in  $\text{H}_2$ . Alternatively, the ratio



may be maintained at a low value by removing the  $\text{H}_2\text{S}$  from the vapor state as quickly as it is formed. The removal of  $\text{H}_2\text{S}$  from the vapor state can be accomplished by providing in a desulfurization zone a solid acceptor which has a greater affinity for hydrogen sulfide than those materials with which the sulfur is bound in the carbonaceous solid fuels. A preferred solid acceptor is one containing manganese oxide, impregnated on an inert carrier. Suitable carrier materials include silica, alumina and silica-alumina preferably in the form of mullite (containing 75 to 85 percent alumina and the balance silica).

Acceptors containing manganese oxide are preferably prepared by soaking the inert carrier particles in an aqueous solution of a soluble manganese salt which thermally decomposes to leave a residue of manganese oxide. Manganese nitrate is a preferred soluble salt for this purpose. The concentration of the aqueous solution should be sufficient to deposit up to about 10 percent by weight of manganese on the carrier. The soaked carrier thereafter is heated to achieve dehydration and decomposition of the deposited manganese salt to the manganese oxide residue. The resulting acceptor should contain up to about 10 percent by weight of manganese, preferably from about 4 to about 8 percent.

Throughout the specification, the term "manganese oxide" refers to compounds containing manganese and oxygen, such as  $\text{MnO}$ ,  $\text{Mn}_3\text{O}_4$ ,  $\text{Mn}_2\text{O}_3$ ,  $\text{MnO}_2$  which compounds are principally in the form of  $\text{MnO}$ . The term "higher oxides of manganese" refers to compounds containing more than one atom of oxygen per atom of manganese, e.g.,  $\text{Mn}_3\text{O}_4$ ,  $\text{Mn}_2\text{O}_3$ ,  $\text{MnO}_2$ .

The reaction of the manganese oxide in the desulfurization treatment is as follows:



Thus the manganese oxide combines with the generated hydrogen sulfide to form manganese sulfide thereby re-

moving from the vapor phase the hydrogen sulfide formed by desulfurization of the carbonaceous solid fuel.

Following sufficient desulfurizing treatment of the carbonaceous solid fuels, the desulfurized fuels are separated from the solid acceptor and recovered as a low sulfur carbonaceous fuel product. As such, the low sulfur carbonaceous solid fuels are suitable for use as metallurgical fuels.

The separated sulfided acceptor is regenerated by treatment with air to restore the manganese oxide for reuse as follows:



Thus in the overall process, the sulfur removed from the carbonaceous solid fuels is rejected from the system in the form of sulfur dioxide. So much of the process has been more fully described in the aforementioned application, S.N. 527,705.

The use of  $\text{H}_2\text{S}$  acceptors has been briefly described in relation to desulfurization processes for carbonaceous solid fuels. Such  $\text{H}_2\text{S}$  acceptors also can be used for removing  $\text{H}_2\text{S}$  from any gas stream, regardless of source. For example, elimination of  $\text{H}_2\text{S}$  from petroleum refinery gases, pipeline gas, and the like can be accomplished by passing the gases over an  $\text{H}_2\text{S}$ -acceptor containing manganese oxide. The  $\text{H}_2\text{S}$  will be absorbed by the acceptor and the manganese oxide converted to manganese sulfide. The sulfided acceptor can be regenerated by treatment with air to release sulfur dioxide and restore the manganese oxide.

The phrase " $\text{H}_2\text{S}$ -absorbing conditions" as employed in this specification refers to a non-oxidizing environment containing  $\text{H}_2\text{S}$  at temperatures where a favorable equilibrium exists for the reaction



The preferred temperature range for " $\text{H}_2\text{S}$ -absorbing conditions" is about 1100 to 1600° F. The ability of an acceptor to react with  $\text{H}_2\text{S}$  "under  $\text{H}_2\text{S}$ -absorbing conditions" is an important determinant in the efficiency of the fundamental desulfurization process.

We have found that repeated use of solid acceptors containing manganese oxide impregnated on silica, alumina or silica-alumina carriers results in deactivation of the acceptor. A brief discussion will explain the deactivation phenomenon.

Freshly impregnated acceptor solids will remove hydrogen sulfide gas from a vapor stream in intimate contact therewith at a determinable rate. Subsequent regeneration of the acceptor by reaction with air will restore the manganese oxide. However the regeneration necessarily is conducted at elevated temperatures which bring about the deactivation of the acceptor (under  $\text{H}_2\text{S}$ -absorbing conditions). When the regenerated manganese oxide acceptor is employed to remove hydrogen sulfide from a gas in contact therewith, a lower reaction rate will be observed. Repeated processing of the acceptor through the sulfiding and regenerating processes will result in further deactivation, i.e., a continued lowering in the rate at which the manganese oxide will remove hydrogen sulfide from a gas in contact therewith.

While the regenerated acceptor does not suffer a significant loss in its capacity to absorb hydrogen sulfide, there is nevertheless a lowering in the rate at which the absorption of hydrogen sulfide occurs. Hence a distinction is made between

(a) The capacity of a regenerated acceptor to absorb hydrogen sulfide and

(b) The rate at which a regenerated acceptor will absorb hydrogen sulfide.

The capacity for hydrogen sulfide absorption depends upon the quantity of manganese oxide present, whereas the rate at which hydrogen sulfide can be absorbed depends upon a condition which is referred to herein as the acceptor's activity under  $\text{H}_2\text{S}$ -absorbing conditions. Hence the term deactivation refers to a lowering of this

activity and the term reactivation refers to an increasing of this activity.

Note that it is possible to have a fully regenerated acceptor (one in which all of the manganese sulfide has been converted to manganese oxide) although that acceptor is deactivated, i.e., the regenerated acceptor will absorb  $H_2S$  only at a diminished rate. Should such a regenerated (deactivated) acceptor be exposed to  $H_2S$ -absorbing conditions for a sufficiently long period of time, the quantity of  $H_2S$  absorbed by it would depend solely on the quantity of manganese oxide which it contains. A reactivated, regenerated acceptor, on the other hand, would absorb the same quantity of  $H_2S$  in a shorter period of time.

It is believed that this deactivation of manganese oxide impregnated carriers results from a physical migration of the manganese into the carrier itself. The penetration of the manganese into the carrier may sometimes be accompanied by chemical reaction resulting in the formation of manganese silicates and aluminates. Any manganese thus converted is removed from the cyclic  $MnO$ - $MnS$ - $MnO$ - $MnS$  et cetera reactions.

The principal object of the present invention is to provide a process for reactivating a manganese impregnated acceptor which has been deactivated. A further object is to provide a regeneration process for converting the manganese sulfide of a manganese impregnated acceptor to the desired manganese oxide with minimum deactivation of the acceptor. A still further object is to provide a desulfurization process which employs manganese impregnated acceptors which can be recirculated throughout the process through sequential sulfur absorbing and sulfur elimination without severe loss of activity (under  $H_2S$ -absorbing conditions).

According to the present invention, a portion of recirculating sulfided acceptor is regenerated and reactivated independently of the portion of recirculating sulfided acceptor. That portion which is both regenerated and reactivated is intimately contacted with an overwhelming excess of oxygen at a temperature of 1000 to 1600° F. to convert substantially all of the manganese in that minor portion to higher oxide forms such as  $Mn_3O_4$  and  $Mn_2O_3$ .

When subsequently reduced to the  $MnO$  form, the acceptor possesses an increased activity (under  $H_2S$ -absorbing conditions). The acceptor which has been subjected to the extensive oxidation preferably is thereafter reduced substantially to  $MnO$  before re-entering the recirculating acceptor stream. We prefer to reduce the reactivated acceptor in a second reactivation treatment by transferring the excess oxygen to a portion of sulfided acceptor also withdrawn from the recirculating acceptor stream.



From the equations, it is seen that only a relatively small quantity of the sulfided acceptor is required to effect the desired transfer of excess oxygen.

Manganese oxide exists in nature in the form of  $MnO_2$  inter alia. It is possible to reduce the  $MnO_2$  to lower oxides as follows:



The complete reduction train is not reversible since the  $MnO_2$  form cannot be restored through ordinary oxidation alone. However, it is possible through oxidation alone to reverse the reaction as follows:



For the purpose of the present invention, it is sufficient that the conversion of acceptor to oxides higher than  $MnO$  be maximized to offset the deactivation phenomenon. The sulfided acceptor contains essentially  $MnS$  and  $MnO$  prior to the reactivation treatment. In

the presence of excess air, the following reactions proceed simultaneously.



Some manganese sulfate may be formed as an intermediate during the oxidation, but it is quickly decomposed 10 autogenously to the oxide:



Thus substantially all of the sulfur contained in the acceptor is eliminated during the first stage reactivation 15 treatment so that the treatment provides full regeneration. In addition, the formation of higher oxides of manganese accomplish a reactivation of the acceptor (under  $H_2S$ -absorbing conditions). While the described reactivation treatment does not fully restore the activity (under  $H_2S$ -absorbing conditions) of the regenerated acceptor, nevertheless, a significant increase in activity is achieved. Maximum activity is not required in most carbon desulfurization processes since an overwhelming excess of acceptor is employed in order to supply the 20 heat required in the desulfurization zone.

Normally, a small quantity of carbonaceous material 25 will be commingled with the sulfided acceptor recovered from the desulfurization zone. This carbonaceous material will be transferred from the desulfurization zone to the reactivation zone to supply the heat requirements via combustion.

For a full understanding of the present invention, its objects and advantages, reference should be had to the following detailed description and accompanying drawings in which:

Figure 1 is a schematic flow diagram illustrating a desulfurization process for carbonaceous solid fuels employing solid acceptors for hydrogen sulfide;

Figure 2 is a schematic flow diagram illustrating the 30 reactivation process steps embodied in the present invention; and

Figure 3 is a graphical representation of the activity loss for manganese oxide-type acceptors according to length of exposure to elevated temperatures.

The generalized flow sheet of Figure 1 illustrates the 45 manner in which an acceptor desulfurization process can be carried out in a continuous manner. A desulfurization zone 10 receives non-caking carbonaceous solids containing sulfur through a conduit 11 and regenerated acceptor solids through a conduit 12. In this instance, the active ingredient of the acceptor solids is manganese oxide. A hydrogen-rich treating gas consisting essentially of hydrogen is introduced into the desulfurization zone 10 through a conduit 13. Additional gases, consisting of hydrogen gas, are autogenously produced through devolatilization of the carbonaceous solids at the elevated 50 temperature of the desulfurization zone 10. Under preferred operating conditions the autogenously produced devolatilization gases will be in sufficient quantity to provide the full hydrogen requirements for desulfurization so that extrinsic hydrogen production is not required.

The desulfurization zone 10 is maintained at a temperature from about 1100 to about 1600° F. Below 55 about 1100° F., the desulfurization rate is low. Operation above about 1600° F. requires excessive heat and also promotes rapid deactivation of the acceptor. The pressure level preferably is high enough to provide a hydrogen gas partial pressure of at least one atmosphere. A total pressure of from one to six atmospheres is preferred.

A typical char (containing sulfur) produced by fluidized 60 carbonization of Pittsburgh Seam coal at 950° F. yields devolatilization gases containing 58.6 percent hydrogen and 24.8 percent methane at 1.3 atmospheres and 1350° F. The same char yields devolatilization gases contain-

ing 48.7 percent hydrogen and 32.9 percent methane at 3 atmospheres and 1350° F.

During passage through the desulfurization zone 10, the treating gases remove sulfur from the carbonaceous solid fuels



forming hydrogen sulfide.

The  $H_2S$ , upon formation, is at once absorbed by the solid acceptor and removed from the gas phase.



Gases are recovered from the desulfurization zone 10 through a conduit 14 and recirculated through conduit 13 for further contact with carbonaceous solids undergoing desulfurization. A net product gas is removed through a conduit 15.

The required residence of carbonaceous solids in the desulfurization zone 10 depends upon the lability of the contaminating sulfur and also upon the level of desulfurization desired. It must be borne in mind that the ultimate sulfur level of the product is determined by the level of  $H_2S$  concentration which the manganese oxide will maintain. Where the hydrogen partial pressure of the treating gases is about one atmosphere or greater, satisfactory desulfurization can be achieved by subjecting the carbonaceous solids to the desulfurization conditions for a period of about three hours or less. Increased absolute pressure, as already pointed out, promotes more rapid desulfurization.

Desulfurized carbonaceous solids are removed from the desulfurization zone 10 as product through a conduit 16. Sulfided acceptor is removed through a conduit 17 and passed to an acceptor regeneration zone 18. Air is introduced into the regeneration zone 18 through a conduit 19 to raise the temperature of the acceptor through combustion of sulfur along with a portion of the carbonaceous solids commingled therewith and to remove sulfur therefrom through oxidation to sulfur dioxide.



The temperature within the regeneration zone 18 is maintained at about 1300 to 1600° F. Hot flue gases containing sulfur dioxide are removed from the regeneration zone 18 through a conduit 20.

Excessive oxidation in the regeneration zone 18 should be avoided in order to restrict the quantity of higher oxides of manganese produced. Ideally, some of the acceptor solids recovered from the regeneration zone 18 should be in the form of  $MnS$ . By maintaining from about 2 to about 15 percent of the manganese as  $MnS$  after regeneration, the oxides of manganese can be maintained principally in the form of  $MnO$  rather than as higher oxides such as  $Mn_3O_4$  or  $Mn_2O_3$ . The presence of higher oxides of manganese in the desulfurization zone undesirably consumes hydrogen gas without accompanying sulfur removal as will be hereinafter described. In general, the amount of oxygen used in the regeneration zone 18 should be within about 20 percent of the stoichiometric quantity, which would be required for oxidizing all of the  $MnS$  to  $MnO$  according to the equation above.

Regenerated acceptor is returned to the desulfurization zone 10 through the conduit 12 without deliberate cooling to serve therein as a means for removing  $H_2S$  therefrom and to supply the heat requirements thereof.

When the desulfurization process is operated as described with an acceptor comprising manganese oxide impregnated on an inert carrier, deactivation of the acceptor will occur as a result of its thermal exposure. According to the present process as illustrated in Figure 2, the acceptor deactivation may be retarded. In Figure 2, the elements of the process relating to the desulfurization stage bear numerals corresponding to those of Figure 1. Corresponding numerals identify corresponding elements. Regenerated acceptor solids are introduced into the desulfurization stage 10 through a conduit 12.

Sulfided acceptor solids comprising inert carriers containing manganese sulfide and manganese oxide are recovered from the desulfurization stage 10 through a conduit 17. A portion of the sulfided acceptor is regenerated in the usual

5 manner by treatment with air at about 1300 to 1600° F. in the regeneration zone 18. Another portion of the recirculating sulfided acceptor is withdrawn through the conduit 21 and transported as a suspension in air (from a conduit 22) through a conduit 23 into a first reactivation vessel 24. The acceptor is maintained in intimate contact with oxygen within the reactivation vessel 24 preferably in the fluidized state with air as a fluidizing gas. The first reactivation vessel 24 is maintained at a temperature of 1000 to 1600° F. The pressure is preferably that maintained in the desulfurization zone 10. The acceptor solids remain in the first reactivation vessel 24 for a sufficient period, from about 5 minutes to several hours, to achieve substantially complete conversion of all the manganese to a higher oxide form. Any manganese sulfide entering the first reactivation vessel 24 will be converted into an oxide of manganese and will form sulfur dioxide. The spent gases, including sulfur dioxide and oxygen-depleted fluidizing gas, are removed through a conduit 25. Usually sufficient carbonaceous fuel will be

20 commingled with the recirculating sulfided acceptor to provide the heat requirements of the first reactivation vessel 24 via combustion in the oxidizing environment therein.

A substantial excess of oxygen is supplied to the first 30 reactivation vessel 24 over that determined by the stoichiometry of the reaction.



Preferably an oxygen excess from about five-fold to about 35 fifty-fold is provided to assure maximum oxidation of the manganese of the acceptor.

The quantity of acceptor subjected to the reactivation treatment of this invention is quite small in relation to the total recirculating stream of sulfided acceptor. In general, from about 1 to about 10 percent of the sulfided acceptor recovered from the desulfurization zone 10 will be reactivated. The major portion of sulfided acceptor recovered from the desulfurization zone 10, preferably more than 90 percent, will be regenerated in the regeneration zone 18 as already described.

45 40 The regenerated, reactivated acceptor solids are withdrawn from the first reactivation vessel 24 principally as higher oxides of manganese through a conduit 26 for reuse in the process. The reactivated, regenerated acceptor solids from conduit 26 may be introduced into the conduit 12 (containing the major portion of regenerated acceptor solids) for reintroduction into the recirculating stream of acceptor solids. This procedure is undesirable since the higher oxides of manganese are immediately reduced to  $MnO$  on entry into the hydrogen-rich environment within the desulfurization zone 10:



50 60 Consumption of valuable hydrogen gas in this manner is inefficient since there is no accompanying desulfurization. Moreover, the reduction of these higher oxides generates water vapor which has a tendency to suppress the fundamental  $H_2S$ -absorbing reaction:



65 The equilibrium for the  $H_2S$ -absorbing reaction is a function of



70 75 in the surrounding vapor. An increase in the partial pressure of water tends to retard the rate at which further  $H_2S$  can be absorbed. Where the minor portion undergoing reactivation according to the present invention amounts to only a few percent of the total recirculating

acceptor stream, the net hydrogen loss may be insignificant.

We prefer to provide a reducing treatment for the highly oxidized acceptor resulting from the first stage of reactivation. The preferred reducing treatment is accomplished by transferring excess oxygen from the reactivated acceptor (containing higher oxides of manganese) to sulfided unregenerated acceptor (containing MnS)



The reducing treatment is carried out in a second reactivation vessel 30.

Accordingly, the reactivated acceptor containing higher oxides of manganese is withdrawn from conduit 26 through a conduit 27. A stoichiometric quantity of sulfided acceptor containing manganese sulfide is withdrawn from the conduit 17 through a conduit 28. Both acceptor streams are joined and introduced through a conduit 29 into a reaction vessel 30. A gas, preferably non-oxidizing, is introduced into the vessel 30 through the conduit 29 to fluidize the bed of acceptor therein and provide intimate contacting conditions. The fluidizing gas should be free of sulfur compounds. Air may be used for this purpose, although an inert flue gas is preferred. Within the second reactivation vessel 30, the reactivated acceptor is reduced and the sulfided acceptor is regenerated as described.

Spent fluidizing gas containing SO<sub>2</sub> is removed from the second reactivation vessel 30 through a conduit 31. The reaction between MnS and higher oxides of manganese is quite rapid, indicating the great affinity of MnS for reacting with oxygen. A residence time of the acceptor within the second reactivation vessel 30 of from a few minutes to several hours is satisfactory. Thus treated acceptor, principally as MnO, is withdrawn from the second reactivation vessel 30 through a conduit 32. In its reactivated, regenerated form, the acceptor from conduit 32 may be introduced directly into the desulfurization zone 10 through the conduit 12. The second reactivation vessel 30 is preferably maintained at a temperature of about 1300 to 1700° F.

The relative quantities of reactivated acceptor and sulfided acceptor interacting in the second reactivation vessel 30 can be calculated from the following generalized equation in which X refers to the ratio of oxide-form oxygen to manganese in the acceptor:



Alternatively, the second reactivation vessel 30 may be eliminated and the reactivated acceptor may be reduced directly in the regeneration vessel 18. According to this alternative embodiment, the reactivated acceptor (containing higher oxides of manganese) is recovered from the first reactivation vessel 24 through the conduit 26 and transferred directly to the regeneration zone 18 through a conduit 33. Interaction between the sulfided acceptor and the reactivated acceptor occurs in the regeneration vessel 18. Since the quantity of higher oxides of manganese in the regeneration zone 18 will be small (about 1 to 10 percent) in contrast to the quantity of sulfided acceptor (about 90 to 99 percent), the bulk of regeneration will continue to occur therein via oxidation as already described.

Figure 3 graphically illustrates the effect of thermal exposure on loss of activity of acceptors impregnated with manganese oxide.

To calculate activity of an acceptor, a weighed batch of the acceptor is placed in a container adapted to confine the acceptor in a bed under fluidizing conditions. A stream of gas having a predetermined composition of hydrogen and H<sub>2</sub>S is passed upwardly through the bed of acceptor at a predetermined constant rate as a

fluidizing gas. Usually the gas contains about 0.7 percent H<sub>2</sub>S in hydrogen. The fraction of entering H<sub>2</sub>S which reacts with the acceptor is measured. Initially substantially all of the entering H<sub>2</sub>S reacts with the acceptor.



For each mol of H<sub>2</sub>S reacted, one mol of water is formed. Thus the amount of water in the effluent gas is a direct measure of the H<sub>2</sub>S reaction.

As a standard measurement, the activity of an acceptor is calculated at that instant when only 90 percent of the entering H<sub>2</sub>S reacts with the acceptor in the batch fluidized bed. The activity is expressed as

$$\frac{\text{grams of H}_2\text{S reacted per hour}}{\text{grams of unreacted MnO in the acceptor bed}}$$

A freshly prepared acceptor has an activity which can be expressed as unity. The measured activity of any other acceptor under investigation can be compared with that of the freshly prepared acceptor (expressed as unity).

To develop the curves of Figure 3, a mullite carrier impregnated with manganese oxide was used. The carrier contained 4 percent of manganese. Samples of the acceptor were exposed to elevated temperatures for varying periods of time to illustrate the effect of thermal exposure on activity loss. The activity of each sample was determined and compared with that of a freshly prepared acceptor. The activity values (expressed as a percentage of the fresh acceptor activity) are presented graphically in Figure 3 for each temperature level of thermal exposure.

The time required for a 50 percent loss in activity would be about 5 hours at 1600° F., about 6 hours at 1500° F., about 87 hours at 1400° F. and about 210 hours at 1350° F. Since the desulfurization processes are operated with an overwhelming excess of acceptor material, maintenance of a maximum activity level is not requisite. Accordingly, full restoration of activity is not required during each regeneration cycle. Thus only a small portion of the recirculating stream of acceptor is subjected to the reactivating treatment of the present invention. For example, from about 1 to 10 percent by weight of the acceptor solids undergoing regeneration would be exposed to the reactivation treatment of this invention.

To illustrate the efficacy of reactivation of the present process, an acceptor was selected comprising a mullite carrier containing 4.02 percent by weight of manganese.

By virtue of extensive thermal treatment, this acceptor had an activity (under H<sub>2</sub>S-absorbing conditions) only 45 percent of its original activity (under H<sub>2</sub>S-absorbing conditions). About 94 percent of the manganese in the acceptor was in the form of manganese sulfide.

Example 1.—To illustrate efficacy of first reactivation stage

The deactivated sulfided acceptor was maintained in a fluidized state at 1000° F. for two hours by passing oxygen gas upwardly therethrough at a partial pressure of one atmosphere oxygen. The acceptor thereafter contained manganese substantially entirely as Mn<sub>2</sub>O<sub>3</sub>.

This acceptor was reduced in a hydrogen atmosphere at 1350° F. to restore the manganese to the MnO form. The reduced, reactivated acceptor thereafter had an activity (under H<sub>2</sub>S-absorbing conditions) about 73 percent of its original activity (when freshly prepared).

Example 2.—To illustrate efficacy of second reactivation stage

An acceptor containing manganese oxide was reactivated via the described oxidation to a composition MnO<sub>1.265</sub>, indicating the presence of higher oxides of manganese, and simulating the reactivated acceptor in the conduit 26. A sulfided acceptor was obtained in

which 2.24 percent of the MnO had been converted to MnS, simulating the sulfided acceptor in the conduit 28. The two ingredients were mixed. The sulfided acceptor contained 12.00 grams of MnO and 0.337 gram of MnS. The reactivated acceptor contained 2.50 grams of MnO<sub>1.265</sub>. The mixture was fluidized at 1650° F. by passing nitrogen gas therethrough for two minutes. The loss in weight of 0.189 gram was exactly that predicted from the equation



where X had a value of 1.265. The resulting acceptor mixture contained manganese substantially entirely as MnO.

According to the provisions of the patent statutes, we have explained the principle, preferred construction, and mode of operation of our invention and have illustrated and described what we now consider to represent its best embodiment. However, we desire to have it understood that, within the scope of the appended claims, the invention may be practiced otherwise than as specifically illustrated and described.

We claim:

1. In a process employing solid acceptors for hydrogen sulfide comprising manganese oxide impregnated on an inert support for absorbing hydrogen sulfide at temperatures above about 1100° F. to form manganese sulfide, followed by oxidizing the manganese sulfide to manganese oxide by reaction with oxygen at elevated temperatures above about 1300° F., wherein the acceptors suffer a decrease in H<sub>2</sub>S-absorbing activity following said oxidizing, the improvement which minimizes loss of the acceptors' activity under H<sub>2</sub>S-absorbing conditions, comprising intimately contacting a minor portion of the manganese sulfide-containing sulfided acceptors with excess oxygen at a temperature of 1000 to 1600° F., converting thereby substantially all of the contacted manganese sulfide to higher oxides of manganese and thereafter recovering the thus-treated acceptors containing higher oxides of manganese reducible to manganese oxide having an increased H<sub>2</sub>S-absorbing activity.
2. The improvement of claim 1 wherein the inert support is selected from the class consisting of silica, alumina and silica-alumina.
3. The improvement of claim 1 wherein the inert support is mullite.
4. In a process employing solid acceptors for hydrogen sulfide comprising manganese oxide impregnated on an inert support for absorbing hydrogen sulfide at temperatures above about 1100° F. to form manganese sulfide, followed by oxidizing the manganese sulfide to manganese oxide by reaction with oxygen at elevated temperatures above about 1300° F., wherein the acceptors suffer a decrease in H<sub>2</sub>S-absorbing activity following said oxidizing, the improvement which minimizes loss of the acceptors' activity under H<sub>2</sub>S-absorbing conditions, comprising intimately contacting a major portion of the sulfided acceptors with oxygen at a temperature of 1300 to 1600° F. to convert substantially all of the contacted manganese sulfide to manganese oxide, contacting a minor portion of the manganese sulfide-containing sulfided acceptors with excess oxygen at a temperature of 1000 to 1600° F., converting thereby substantially all of the thus-contacted manganese sulfide to higher oxides of manganese, thereafter recovering the thus-treated minor portion containing higher oxides of manganese reducible to manganese oxide having an increased H<sub>2</sub>S-absorbing activity and recombining with said major portion.
5. In a process employing solid acceptors for hydrogen sulfide comprising manganese oxide impregnated on an inert support for absorbing hydrogen sulfide at temperatures above about 1100° F. to form manganese sulfide, followed by oxidizing the manganese sulfide to manganese oxide by reaction with oxygen at elevated temperatures above about 1300° F., wherein the acceptors suffer a decrease in H<sub>2</sub>S-absorbing activity following said oxidizing, the improvement which minimizes loss of the acceptors' activity under H<sub>2</sub>S-absorbing conditions, comprising intimately contacting a major portion of the sulfided acceptors with oxygen in a regenera-

peratures above about 1100° F. to form manganese sulfide, followed by oxidizing the manganese sulfide to manganese oxide by reaction with oxygen at elevated temperatures above about 1300° F., wherein the acceptors suffer a decrease in H<sub>2</sub>S-absorbing activity following said oxidizing, the improvement which minimizes loss of the acceptors' activity under H<sub>2</sub>S-absorbing conditions, comprising intimately contacting a major portion of the sulfided acceptors with oxygen at a temperature of 1300 to 1600° F. to convert substantially all of the contacted manganese sulfide to manganese oxide, contacting a first minor portion of the manganese sulfide-containing sulfided acceptors with excess oxygen at a temperature of 1000 to 1600° F., converting thereby substantially all of the thus-contacted manganese sulfide to higher oxides of manganese, thereafter contacting a second minor portion of the sulfided acceptors with the thus-treated first minor portion at a temperature of 1300 to 1700° F. whereby the manganese sulfide of said second minor portion is converted to manganese oxide by reaction with oxygen released from said first minor portion whose higher oxides of manganese are converted substantially to manganese oxide, recovering the thus-treated first and second minor portions containing manganese oxide having an increased H<sub>2</sub>S-absorbing activity and recombining with said major portion.

6. In the method of removing sulfur from particulate carbonized carbonaceous solids, which comprises preparing an intimate admixture of said carbonaceous solids and particulate acceptor solids comprising inert carriers having manganese oxide impregnated thereon, subjecting said admixture to treatment at a temperature above 1100° F. in the presence of hydrogen gas until a portion of the initial sulfur has been removed from said carbonaceous solids and transferred to said acceptor solids forming manganese sulfide, separating particulate acceptor solids containing manganese sulfide from low sulfur carbonaceous solids, recovering low sulfur particulate carbonaceous solids as product, and restoring the H<sub>2</sub>S-absorbing property of sulfided acceptor solids for recirculation in the process, the improvement in the last-mentioned step comprising contacting a major portion of said sulfided acceptor solids at a temperature of 1300 to 1600° F. under oxidative conditions to remove sulfide sulfur therefrom and reform manganese oxide thereby, contacting a minor portion of said sulfided acceptor solids at a temperature of 1000 to 1600° F. with excess oxygen to convert substantially all of the manganese sulfide to higher oxides of manganese, thereafter reducing the higher oxides of manganese in said minor portion substantially to manganese oxide, and recombining the thus-treated minor portion with the treated major portion for repeated admixing and processing with said particulate carbonized carbonaceous solids.

7. The method of claim 6 wherein the particulate carbonized carbonaceous solids are carbonaceous briquets and the inert carriers comprise finely divided fluidizable size particles of an inert material selected from the class consisting of silica, alumina and silica-alumina.

8. The method of claim 6 wherein the particulate carbonized carbonaceous solids comprise char produced by fluidized low temperature carbonization of caking bituminous coal.

9. In a process employing solid acceptors for hydrogen sulfide comprising manganese oxide impregnated on an inert support for absorbing hydrogen sulfide at temperatures above about 1100° F. to form manganese sulfide, followed by oxidizing the manganese sulfide to manganese oxide by reaction with oxygen at elevated temperatures above about 1300° F., wherein the acceptors suffer a decrease in H<sub>2</sub>S-absorbing activity following said oxidizing, the improvement which minimizes loss of the acceptors' activity under H<sub>2</sub>S-absorbing conditions, comprising intimately contacting a major portion of the sulfided acceptors with oxygen in a regenera-

tion zone at a temperature of 1300 to 1600° F. to convert substantially all of the contacted manganese sulfide to manganese oxide, contacting a minor portion of the manganese sulfide-containing sulfided acceptors with excess oxygen at a temperature of 1000 to 1600° F., converting thereby substantially all of the thus-converted manganese sulfide to higher oxides of manganese, thereafter introducing the thus-treated minor portion into said regeneration zone to reduce said higher oxides of manganese substantially to manganese oxide and recovering from said regeneration zone, in admixture with said major portion, the minor portion containing manganese oxide having an increased H<sub>2</sub>S-absorbing activity.

10. In the method of removing sulfur from particulate carbonized carbonaceous solids, which comprises preparing an intimate admixture of said carbonaceous solids and particulate acceptor solids comprising inert carrier having manganese oxide impregnated thereon, subjecting said admixture to treatment at a temperature above 1100° F. in the presence of hydrogen gas until a portion of the initial sulfur has been removed from said carbonaceous solids and transferred to said acceptor solids forming manganese sulfide, separating particulate acceptor solids containing manganese sulfide from low sulfur carbonaceous solids, recovering said low sulfur particulate carbonaceous solids as product, and restoring the H<sub>2</sub>S-absorbing property of sulfided acceptor solids for recirculation in the process, the improvement in the last-mentioned step comprising contacting a major por-

tion of said sulfided acceptor solids in a regeneration zone at a temperature of 1300 to 1600° F. under oxidative conditions to remove sulfide sulfur therefrom and reform manganese oxide thereby, contacting a minor portion of said sulfided acceptor solids at a temperature of 1000 to 1600° F. with excess oxygen to convert substantially all of the manganese sulfide to higher oxides of manganese, thereafter introducing the thus-treated minor portion into said regeneration zone to reduce said higher oxides of manganese to manganese oxide and recovering from said regeneration zone the thus-treated minor portion containing manganese oxide having an increased H<sub>2</sub>S-absorbing activity in admixture with the treated major portion for repeated admixing and processing with such particulate carbonized carbonaceous solids.

11. The method of claim 10 wherein the particulate carbonized carbonaceous solids are carbonaceous briquets and the inert carriers comprise finely divided fluidizable size particles of an inert material selected from the class consisting of silica, alumina and silica-alumina.

12. The method of claim 10 wherein the particulate carbonized carbonaceous solids comprise char produced by fluidized low temperature carbonization of caking bituminous coal.

References Cited in the file of this patent

UNITED STATES PATENTS

2,824,047 Gorin et al. ----- Feb. 18, 1958